

## UNITED STATES PATENT OFFICE

2,504,927

## PRODUCTION OF ALKALI METAL HYDRIDES

Virgil L. Hansley, Niagara Falls, N. Y., assignor to  
 E. I. du Pont de Nemours & Company, Wil-  
 mington, Del., a corporation of Delaware

No Drawing. Application April 15, 1947,  
 Serial No. 741,699

13 Claims. (Cl. 23—204)

1

This invention relates to the production of alkali metal hydrides.

Freudenberg et al. in U. S. Patent 1,796,265, describe a process for making alkali metal hydrides which involves mixing a molten alkali metal with a finely divided solid inert material and reacting the mixture with hydrogen at an elevated temperature. My U. S. Patent 2,372,671 describes an improvement of that method which involves adding to the mixture of molten metal and finely divided solid inert material a small amount of a hydrocarbon which has at least 8 carbon atoms and is capable of reacting with the alkali metal to form an alkali metal hydrocarbide to facilitate dispersion of molten metal over the inert solid material and thereby increase the rate of hydrogen absorption. Examples of such hydrocarbons are the isomeric cymenes, isopropyl benzene, the isomeric isopropyl naphthalenes, anthracene and the like. Preformed alkali metal hydrocarbides of such hydrocarbons may also be used.

It is an object of the present invention to provide an improved process for producing alkali metal hydrides. A further object is to provide an improvement of the above Freudenberg et al. process. A still further object is a method for preparing such metal hydrides and particularly sodium hydride whereby the rate of reaction is greatly increased with a resulting increase in the space-time yield to obtain alkali metal hydride in a highly reactive, white, finely divided form. Still further objects will be apparent from the ensuing description.

The above objects are accomplished in accordance with the invention by mixing a molten alkali metal with a finely divided solid material and a relatively small amount of a dispersing agent which may be an acetylenic hydrocarbon having the structural group  $-\text{C}\equiv\text{CH}$  or an alkali metal derivative of such a hydrocarbon, and reacting the mixture with hydrogen at a temperature above the melting point of the alkali metal.

As typical of the acetylenic hydrocarbons that may be employed I mention acetylene, methyl acetylene, ethyl acetylene, n-propyl acetylene, isopropyl acetylene, vinyl acetylene and phenyl acetylene. In place of such hydrocarbons, alkali metal derivatives thereof in which the hydrogen in the  $-\text{C}\equiv\text{CH}$  group has been replaced by an alkali metal may be used.

I have discovered that the presence of a hydrocarbon of the above type, or an alkali metal derivative thereof, in the mixture of molten alkali metal and finely divided solid inert material

2

facilitates the dispersion of the alkali metal over the solid material and results in a substantially greater rate of absorption of hydrogen by the reaction to produce the metal hydride. The chemical identity of the agent which actually functions as the dispersing agent is not known. It is known, however, that effective dispersemnt of the sodium may be accomplished by adding either, for example, acetylene or a sodium derivative thereof, such as sodium acetylide ( $\text{NaC}_2\text{H}$ ) or sodium carbide ( $\text{Na}_2\text{C}_2$ ). When either acetylene or sodium acetylide is used, it is probably rapidly converted to sodium carbide. It is not known however, whether the latter functions as the active dispersing agent or is decomposed or adds acetylene under the conditions of use to form the actual active agent. Insofar as the present process is concerned, substantially the same results are achieved whether acetylene, sodium acetylide or sodium carbide, or one of the other above mentioned acetylenic hydrocarbons, is added as suggested. Accordingly, in describing and claiming the invention all such compounds are referred to as "dispersing agents" since they either act per se as the dispersing agent or form the active dispersing agent under the conditions of use.

In carrying out the process, the molten alkali metal and solid inert material may be mixed together with, for example, acetylene, after which the mixture may be subjected to the action of hydrogen. Alternatively, sodium acetylide or sodium carbide may be added to the mixture of metal and solid material prior to or simultaneously with the introduction of hydrogen. A particularly convenient mode of operation involves the addition of hydrogen containing a small amount of acetylene to an agitated mixture of the molten metal and inert solid material. If desired, the acetylene may be added separately from the hydrogen, either continuously or intermittently.

Only a relatively small amount of the dispersing agent need be present in the mixture of molten metal and solid material to effect excellent dispersion of the molten metal over the solid material. Generally, amounts of from 0.05 to about 1% based upon the combined weight of the alkali metal and inert solid material is sufficient to give excellent results. Larger amounts, e. g., up to 10%, may be used but are not recommended.

Sodium hydride prepared by the method of my Patent 2,372,671 tends to be somewhat discolored due apparently to the formation of free carbon resulting from pyrolysis of the dispersing agent employed. Thus, when using p-cymene or other

aromatic hydrocarbon, products having a grayish color are usually formed. In contrast, products prepared in accordance with the present invention using, for example, acetylene as the dispersing agent are white in color. Furthermore, they are much more finely divided than prior products, their particle size ranging from about 1 to 10 microns, as compared with products obtained by my previous method whose particle size generally is 100 microns or greater. The present product is much more reactive for use in catalyzing various organic reactions, e. g., condensations of the Claisen type, and the presence therein of small quantities of the dispersing agent has no deleterious effect.

The invention is further illustrated by the following examples:

*Example 1*

A small cylindrical steel reaction vessel was fitted with a gas inlet and outlet and a conventional thermocouple means for determining temperature within the vessel. The vessel was arranged to rotate horizontally about its axis at about 100 R. P. M. A few small pieces of iron were placed in the vessel to assist in stirring the charge. A constant temperature air bath was arranged around the vessel in order to aid maintaining the desired reaction temperature.

Sufficient preformed sodium hydride to occupy 10-15% of the volume was charged into the vessel while cold, the vessel having previously been filled with nitrogen. The charge was heated to 300-385°C. while rotating the vessel and while passing in a slow stream of hydrogen. An increment of molten sodium was added to the sodium hydride and the passage of hydrogen was continued at such a rate that only a few bubbles escaped per minute while continuing rotation of the vessel and while maintaining the temperature within the vessel at the level indicated. The hydrogen employed contained a small amount of acetylene. When the first increment of sodium had been reacted, another increment was added without intermediate cooling and the cycle repeated. The results tabulated below show the production of sodium hydride going through 10 such cycles or runs. As the reaction vessel filled due to the production of sodium hydride, some of the product was discharged, but sufficient was left in the vessel to constitute a "heel" for the next run. In adding sodium to the hydride "heel" it is not advisable to add more than about 20% by weight of sodium based upon the weight of the "heel."

In the following table, the weights of hydride "heel" at the beginning of several runs are shown along with the rates at which hydrogen was absorbed. In the runs indicated, the amount of acetylene employed varied between about 0.05 and 0.5% based upon the combined weight of the "heel" and the sodium.

| Run | Hydride Heel, g. | O <sub>2</sub> H <sub>2</sub> , Wt. Per Cent | H <sub>2</sub> Absorption, l./min. |
|-----|------------------|----------------------------------------------|------------------------------------|
| A   | 175              | 0.30                                         | 3.2                                |
| B   | 231              | 0.50                                         | 4.2                                |
| C   | 325              | 0.49                                         | 4.0                                |
| D   | 234              | 0.49                                         | 3.4                                |
| E   | 276              | 0.46                                         | 3.0                                |
| F   | 334              | 0.42                                         | 4.2                                |
| G   | 186              | 0.42                                         | 4.0                                |
| H   | 291              | 0.34                                         | 4.0                                |
| I   | 360              | 0.32                                         | 2.8                                |
| J   | 444              | 0.29                                         | 4.3                                |

*Example 2*

This example consists of three cycles or runs carried out as described in Example 1. In place of acetylene, however, p-cymene was employed as the dispersing agent in amounts which varied between 1 to 3% of the weight of the charge.

| Run | Hydride Heel, g. | H <sub>2</sub> Absorption, l./min. |
|-----|------------------|------------------------------------|
| A   | 312              | 1.4                                |
| B   | 354              | 1.5                                |
| C   | 319              | 1.3                                |

The rate of hydrogen absorption was substantially greater in Example 1 than in Example 2, even though p-cymene was employed in the latter case in concentrations much greater than was acetylene. Furthermore, the product obtained in Example 2 had a grayish color, whereas the product of Example 1 was almost pure white. Also, the product of Example 1 was visibly more finely divided and substantially more reactive than the product of Example 2.

My process is suitable for making the hydride of any of the alkali metals, i. e. sodium, potassium, lithium, cesium and rubidium. Mixtures of one or more of the alkali metals may be reacted with hydrogen according to the present process to produce mixtures of alkali metal hydrides.

The hydrogenation reaction may be carried out in accordance with the invention at a temperature just above the melting point of the alkali metal although the rate of reaction at such temperature is low. Temperatures as high as 500 to 600°C. may be used provided sufficient hydrogen pressure is employed to prevent undue decomposition of the hydride product. The preferred temperature range is 200 to 450°C.

The process will generally be carried out at or slightly above atmospheric pressure although pressures substantially above or below atmospheric pressure may be employed if desired. As indicated above, when relatively high temperatures are used pressures above atmospheric will generally be required. Other gases may be introduced with the hydrogen and such gases may be inert diluents or may be reactive gases to produce a mixture of the hydride and another alkali metal compound. For ordinary purposes however, such other gases will not be used and except perhaps for the presence of a small amount of acetylene or other acetylenic hydrocarbon substantially pure hydrogen will generally be employed.

The finely divided inert solid material employed in starting the process as a carrier for the molten alkali metal may be any material such as sand, clay, various powdered metals and the like, including salts which are infusible and inactive towards the reactants present under the conditions of use. I prefer, however, to use preformed alkali metal hydride and particularly preformed alkali metal hydride of the metal which is to be hydrogenated. Thus, in forming sodium hydride, sodium hydride is used as carrier for the molten sodium.

I claim:

1. A method for preparing an alkali metal hydride comprising reacting hydrogen with a mixture of a relatively small amount of an alkali metal and a relatively large amount of a finely divided solid material in the presence of a medium of a reaction product of an alkali metal and

an acetylenic compound, said reaction product having an alkali metal atom directly attached to at least one of two carbon atoms which are directly joined to each other by a triple bond, at a temperature above the melting point of the alkali metal.

2. The method of claim 1, wherein the reaction product of an alkali metal and an acetylenic compound is present in an amount equal to 0.01 to 1% based upon the combined weight of the alkali metal and the solid material.

3. The method of claim 1 wherein the acetylenic compound is acetylene.

4. The method of claim 1 wherein the alkali metal is sodium.

5. The method of claim 4 wherein the temperature is between the melting point of sodium and 600° C.

6. The method of claim 4 wherein the reaction temperature is 200 to 450° C.

7. A method of producing an alkali metal hydride comprising agitating a mixture of an alkali metal and at least 80% by weight of a finely divided inert solid carrier therefor at a temperature between the melting point of said metal and 600° C. in the presence of hydrogen and supplying to said mixture a modicum of an acetylenic hydrocarbon.

8. The method of claim 7 wherein the acetylenic hydrocarbon contains less than 5 carbon atoms.

9. The method of claim 8 wherein the acetylenic hydrocarbon is acetylene and is supplied in an amount equal to 0.05 to 0.5% based on the weight of said mixture.

10. The method of claim 9 wherein the solid carrier is an alkali metal hydride.

11. The method of claim 10, wherein the alkali metal is sodium and the solid carrier is sodium hydride.

12. The method of claim 11 wherein the temperature is 240 to 450° C.

13. A method of producing sodium hydride comprising agitating a mixture of sodium and at least 80% by weight of sodium hydride at a temperature of 240 to 450° C. while supplying to said mixture hydrogen containing 0.05 to 0.5% of acetylene based upon the weight of said mixture.

VIRGIL L. HANSLEY.

REFERENCES CITED

The following references are of record in the file of this patent:

UNITED STATES PATENTS

| Number    | Name       | Date         |
|-----------|------------|--------------|
| 1,958,012 | Muckenfuss | May 8, 1934  |
| 2,372,670 | Hansley    | Apr. 3, 1945 |
| 2,372,671 | Hansley    | Apr. 3, 1945 |